

# UNITED STATES PATENT OFFICE.

AMBROSE H. ROSENTHAL, OF SALEM, MASSACHUSETTS.

## ART OF TREATING LEATHER.

No Drawing.

Application filed September 12, 1925. Serial No. 56,088.

My invention relates generally to the art of treating leather and refers more especially to a process of imparting a metallic appearance to ordinary leather, patent leather or imitation leather.

In carrying my invention into practice, I first apply to the leather a coating of a bismuth combination such as a coating of bismuth oxychloride which may be either in 10 the form of powder or in the form of a solution in alcohol or water. The bismuth oxychloride is well rubbed into the leather and the latter is polished until smooth.

I next apply to the thus treated leather 15 surface, a coating of cellulose i. e. gun cotton in solution, preferably acetone. This may be sprayed or flowed onto the leather surface and is permitted to dry thereon. The cellulose solution may have incorporated 20 therein the desired color or metallic shade which is to be imparted to the leather.

As an alternative to incorporating the color in the cellulose solution, a basic color i. e. one soluble in alcohol may be applied to 25 the treated surface after the cellulose solu-

tion has been applied and has become dry.

I may, at this stage, apply another coating of bismuth oxychloride, in solution, the result of which will be to produce relatively light colors.

For the purpose of protecting the leather surface, treated as above described, against deterioration I find it desirable to apply thereto a coating of a flexible varnish, such as cellulose varnish or the like.

It will be understood that the term "leather" as used in the foregoing specification and in the appended claim is intended to include real leather, patent leather and imitation or artificial leather.

I claim:

A method of treating leather, which consists in applying thereto a coating of bismuth oxychloride in solution, a coating of cellulose solution, a coloring medium, a second bismuth oxychloride solution, and a flexible varnish.

In testimony whereof I affix my signature.

AMBROSE H. ROSENTHAL.